# EUROPEAN PATENT SPECIFICATION

(11) **EP 2 272 997 B1**
(45) Date of publication and mention of the grant of the patent: **17.04.2013**
(21) Application number: 10166735.0
(22) Date of filing: 22.06.2010
(51) Int. Cl.: C23C 18/28, C23C 18/30

(54) **Colloidal palladium activator composition and preparation method**
Kolloidale Palladium Aktivatorlösung und Herstellungsverfahren
Composition d'activation de palladium colloïdale et procédé de préparation

(30) Priority: 22.06.2009 CN 200910108122
(43) Date of publication of application: 12.01.2011
(73) Proprietor: BYD Company Limited, Shenzhen 518118 (CN)
(72) Inventor: GONG, Qing, 518118, Shenzhen (CN); WEI, Jialiang, 518118, Shenzhen (CN); LIAN, Junlan, 518118, Shenzhen (CN)
(74) Representative: Gulde Hengelhaupt Ziebig & Schneider

(56) References cited:
- WO-A2-03/033764
- US-A- 4 933 010

## Description

The present disclosure relates to a colloidal palladium activator composition for chemical plating on the surface of a resin and a preparation method thereof. The disclosure further refers to a corresponding activation method for nonmetal surfaces.

### BACKGROUND OF THE PRESENT DISCLOSURE

Nonmetal materials are often nonconductive, so membranes must be applied to them before plating. One of the most common plating methods is electroless plating, which absorbs a number of active centers in the surface of the nonmetal material by activation pretreatments, then forms the initiation of the electroless plating. Activation has a significant influence on the quality of the plated layers.

Acid colloidal palladium activators have long activating lives, however, it not only requires complex preparation processes, but also can easily fail in outside condition which may result in short lives. In addition, acid compositions in the activators may harm people's health, and corrode the substrate. Through adding chloride elements in colloidal palladium, like sodium chloride, Shipley Company, L.L.C. obtained a base colloidal palladium activator with long life and no hydrochloride mist.

Patent No. US 4933010 disclosed a sensitizing activator comprising stannous chloride, palladium chloride, and sodium chloride. The sensitizing activator may further comprise vanillin. The sensitizing activator may prevent the occurrence of hydrochloride mist, and increase the absorbing amount of the colloidal palladium particles through the vanillin's enhancement on the adhesive strength between the colloidal palladium and the substrate. The activator has poor stability.

### SUMMARY OF THE PRESENT DISCLOSURE

According to one aspect of the present disclosure there is provided a colloidal palladium activator composition comprising colloidal palladium particles, sodium chloride, glyoxylic acid, hydrochloride solution, stannous chloride, and a stabilizer.

According to another aspect of the present disclosure there is provided a method for preparing the colloidal palladium composition comprising the steps of: dispersing hydrochloride solution, stannous chloride, glyoxylic acid, and a stabilizer into a sodium chloride solution to prepare an A solution; dispersing a palladium sodium into a hydrochloride solution and adding stannous chloride to prepare a B solution; mixing the A and B solution to form the colloidal palladium activator.

According to yet another aspect of the present disclosure there is provided an activating method for a nonmetal surface comprises contacting a nonmetal substrate under pretreatment with the colloidal palladium activator composition to form a nonmetal substrate containing a number of active centers.

The glyoxylic acid has strong reductive ability, which may prevent the oxidation of Pd²⁺ in the activator to prolong the life of the activator. At the same time, the glyoxylic acid distributes around the colloidal palladium particles which may separate the colloidal palladium particles more evenly and prevent the colloidal palladium particles from coagulation, further strengthening the activity of the activator. The present disclosure also discloses a method for preparing colloidal palladium particles. During the activating process according to an embodiment of the present disclosure, glyoxylic acid may absorb on the surface of the nonmetal substrate at first to strengthen the bonding force between the glyoxylic acid and the nonmetal substrate, which may favor the evenness and flatness of the coating layer, and further enhance the adhesive strength between the plating layer and the substrate.

### DETAILED DESCRIPTION OF THE EMBODIMENT

According to a first aspect of the present disclosure, there is provided a colloidal palladium activator composition comprising colloidal palladium particles, sodium chloride, glyoxylic acid, hydrochloride solution, stannous chloride, and a stabilizer.

The colloidal palladium activator composition comprises colloidal palladium particles, which may absorb in the surface of the nonmetal substrate, in particular made of a nonconductive resin, and forms a number of active centers to metalize the surface of the nonmetal substrate.

The colloidal palladium activator composition comprises sodium chloride, the sodium chloride forming a complex compound with the colloidal palladium particles to disperse the colloidal palladium particles evenly in the activator. In addition, the containing of sodium chloride may further reduce the amount of hydrochloride, to prevent the occurrence of hydrochloride mist.

The colloidal palladium activator composition comprises hydrochloride for adjusting the PH value of the activator. Further, the hydrogen and chloride may stabilize the Sn²⁺ in the activator, making it not easy to hydrolysis and oxidation. The Sn²⁺ may prevent the colloidal from failure.

The colloidal palladium activator composition comprises a stabilizer, which prevents the Sn²⁺ from oxidation to enhance the stability of the activator. In this way, life of the activator is prolonged. The stabilizer is well known to those with ordinary skill in the art, such as one or more selected from a group consisting of sodium stannate, urea, ascorbic acid, and combinations thereof.

The colloidal palladium activator composition comprises glyoxylic acid, which prolongs the life of the activator. In addition, after activated by the activator comprising glyoxylic acid, the nonmetal substrate may achieve a uniform and flat plating layer having high adhesive strength with the substrate. The inventor found that the glyoxylic acid may prolong the life of the activator in following ways: 1) its reductive ability may protect the Sn²⁺ from oxidation to prevent the failure of the activator; 2) the glyoxylic acid may absorb around colloidal palladium particles and charge the colloidal palladium, to make the colloidal palladium particles disperse more uniformly and avoid coagulation of the colloidal palladium particles.

During the activation progress, the state of the absorbing layer depends on the distribution of the active centers in the surface of the nonmetal substrate. An even distribution of the colloid palladium particles, small diameters of the colloid palladium particles may form a small and dense distribution of active centers, which may favor the formation of an even plating layer with a short initiation cycle. According to an embodiment, the colloidal palladium particles have an average diameter of 80 nm to 300 nm.

According to an embodiment, based on the colloidal palladium activator composition, the colloidal palladium particles have concentrations of 0.0002 mol/L to 0.006 mol/L, preferably 0.0004 mol/L to 0.003 mol/L; the sodium chloride has a concentration of 2.567 mol/L to 3.756 mol/L, preferably 2.75 mol/L to 3.60 mol/L; the glyoxylic acid has a concentration of 0.002 mol/L to 0.35 mol/L, preferably 0.01 mol/L to 0.2 mol/L; the hydrochloride solution has a concentration of 0.12 mol/L to 0.96 mol/L, preferably 0.24 mol/L to 0.72 mol/L; the stannous chloride has a concentration of 0.022 mol/L to 0.088 mol/L, preferably 0.031 mol/L to 0.066 mol/L; the stabilizer has a concentration of 0.001 mol/L to 1 mol/L, preferably 0.002 mol/L to 0.8 mol/L.

According to an embodiment, the colloidal palladium activator composition may further comprise a surface wetting agent. The surface wetting agent is well known to those with ordinary skill in the art, such as one or more selected from a group consisting of isopropanol, methanol, ethanol, and combinations thereof. There are no specific concentration limits on the wetting agent. Preferably, the wetting agent may have a concentration of 0.003 mol/L to 0.3 mol/L, more preferably 0.01 mol/L to 0.2 mol/L.

According to an embodiment, the colloidal palladium activator composition may have a PH value of 0.2 to 0.9.

According to another aspect of the disclosure, a method for preparing the colloidal palladium activator composition comprises the steps of: dispersing hydrochloride solution, stannous chloride, glyoxylic acid, and stabilizer into a sodium chloride solution to prepare an A solution; dispersing a palladium sodium into a hydrochloride solution and adding stannous chloride to prepare a B solution; mixing the A and B solution to form the colloidal palladium activator composition.

According to an embodiment, a surface wetting agent may added to the sodium chloride solution, while the surface wetting agent is one of more selected from a group consisting of isopropanol, methanol, ethanol, or the combinations thereof. The stannous chloride and palladium chloride may have a chemical reaction representing by the following formular:

Sn²⁺ + Pd²⁺ → Sn⁴⁺ + Sn⁰

where B solution is prepared. According to an embodiment, the molar ratio of palladium chloride to stannous chloride is less than 1, preferably 0.5. According to an embodiment, the reaction is performed under a temperature of about 20 °C to 40 °C for 10 min to 30 min.

Further, an activation method for a nonmetal surface, like a resin substrate, is disclosed. The method provides a number of active centers in the nonmetal substrate by use of the above mentioned activator composition.

Suitable nonmetal materials for activation are well known to those with ordinary skill in the art, which are hydrophilic after rough treatments, such as Polyimide (PI), acrylonitrile butadiene styrene (ABS resin), and polyethylene terephthalate (PET), with PI as a preferred material.

Pretreatments maybe applied before the activation. The pretreatments are well known to those with ordinary skill in the art, with no special limit. Generally, the pretreatments include grease removal and rough treatments.

The object of grease removal is to removal greases on the surface of the nonmetal substrate. According to an embodiment, grease removal comprises the steps of: immersing the nonmetal substrate in a solution having about 1 mol/L sodium hydroxide, about 1 mol/L sodium carbonate and about 0.1 mol/L sodium dodecyl sulfonate; cleaning the substrate with clean water, where the grease removal progress may not take too long time, for about 10 min to 20 min as preferable. The solution may have a temperature of about 40 °C to 60 °C. The cleaning may first be performed using hot water, then using cold water.

The object of rough treatments is to make the substrate hydrophilic, and to form concavities in the surface of the substrate to favor the activation later on. The rough treatments may vary due to the types of the substrates. In an embodiment, PI surface requires a strong alkli adjusting agent comprising hydrazine hydrate and potassium hydroxide. PI adjusting agents are commercially available, such as SF-01 provided by ZHUHAI SMART ELECTRONIC MATERIAL Co., LTD. Rough treatments for an ABS surface apply a mixture of concentrated sulfuric acid and chromic anhydride. Rough treatments for a PET surface apply a solution include potassium permanganate and sodium hydroxide.

The contact between the substrate and the activator may be performed in room temperature, with no special limit. The contacting temperature is preferable about 20 °C to 30 °C, for about 3 min to 5 min. In this way, deficiencies of the plating layers with uniform thicknesses, which is resulted from the insufficient activation and uniform deposition center in the nonmetal substrate due to insufficient activation time, are addressed. At the same time, issues of insufficient adhesive strength of the plating layers, which are caused by too thick plating layers on the deposition center due to extra long activation time, are addressed.

The nonmetal substrate may be moved to achieve a sufficient activation in the whole surface. In this way, a nonmetal substrate covered by uniform palladium colloidal is obtained.

The activator is only required to immerse the surface of the nonmetal substrate, with no special limit on amounts of the nonmetal substrate and activator.

The following embodiments disclose palladium colloidal activator compositions and their preparation.

### EMBODIMENT 1

3.422 mol sodium chloride were added into 750 ml deionized water to prepare a mixture. The mixture was stirred until dissolution. 0.24 mol concentrated hydrochloride, 0.013 mol glyoxylic acid , 0.020 mol isopropanol, and 0.832 mol urea were added to the mixture and stirred until dissolution to prepare a solution.

0.00028 mol palladium chloride was added in 70 ml deionized water having 0.36 mol concentrated hydrochloride to prepare a mixture. The mixture was stirred until dissolution. 0.00056 mol stannous chloride was added to the mixture and stirred for about 12 min to form a colloidal palladium mixture. The colloidal palladium mixture was added to the solution, and deionized water was added to make the volume of the solution to be 1 L. The solution was placed for about 3 h under a temperature of about 55 °C to prepare a colloidal palladium activator labeled as A1.

### EMBODIMENT 2

3.422 mol sodium chloride were added into 750 ml deionized water to prepare a mixture. The mixture was stirred until dissolution. 0.24 mol concentrated hydrochloride, 0.013 mol glyoxylic acid , 0.2 mol isopropanol, and 0.832 mol urea were added to the mixture and stirred until dissolution to prepare a solution.

0.00028 mol palladium chloride was added in 70 ml deionized water having 0.36 mol concentrated hydrochloride to prepare a mixture. The mixture was stirred until dissolution. 0.00056 mol stannous chloride was added to the mixture and stirred for about 12 min to form a colloidal palladium mixture. The colloidal palladium mixture was added to the solution, and deionized water was added to make the volume of the solution to be 1 L. The solution was placed for about 3 h under a temperature of about 55 °C to prepare a colloidal Palladium activator labeled as A2.

### EMBODIMENT 3

3.422 mol sodium chloride were added into 750 ml deionized water to prepare a mixture. The mixture was stirred until dissolution. 0.24 mol concentrated hydrochloride, 0.005 mol glyoxylic acid , 0.020 mol isopropanol, and 0.832 mol urea were added to the mixture and stirred until dissolution to prepare a solution.

0.00028 mol palladium chloride was added in 70 ml deionized water having 0.36 mol concentrated hydrochloride to prepare a mixture. The mixture was stirred until dissolution. 0.00056 mol stannous chloride was added to the mixture and stirred for about 12 min to form a colloidal palladium mixture. The colloidal palladium mixture was added to the solution, and deionized water was added to make the volume of the solution to be 1 L. The solution was placed for about 3 h under a temperature of about 55 °C to prepare a colloidal palladium activator labeled as A3.

### EMBODIMENT 4

3.422 mol sodium chloride were added into 750 ml deionized water to prepare a mixture. The mixture was stirred until dissolution. 0.24 mol concentrated hydrochloride, 0.013 mol glyoxylic acid , 0.020 mol isopropanol, and 0.832 mol urea were added to the mixture and stirred until dissolution to prepare a solution.

0.00028 mol palladium chloride was added in 70 ml deionized water having 0.36 mol concentrated hydrochloride to prepare a mixture. The mixture was stirred until dissolution. 0.00045 mol stannous chloride was added to the mixture and stirred for about 12 min to form a colloidal palladium mixture. The colloidal palladium mixture was added to the solution, and deionized water was added to make the volume of the solution to be 1 L. The solution was placed for about 3 h under a temperature of about 55 °C to prepare a colloidal palladium activator labeled as A4.

### EMBODIMENT 5

3.422 mol sodium chlorides were added into 750 ml deionized water to prepare a mixture. The mixture was stirred until dissolution. 0.24 mol concentrated hydrochloride, 0.013 mol glyoxylic acid, and 0.832 mol urea were added to the mixture and stirred until dissolution to prepare a solution.

0.00028 mol palladium chloride was added in 70 ml deionized water having 0.36 mol concentrated hydrochloride to prepare a mixture. The mixture was stirred until dissolution. 0.00056 mol stannous chloride was added to the mixture and stirred for about 12 min to form a colloidal palladium mixture. The colloidal palladium mixture was added to the solution, and deionized water was added to make the volume of the solution to be 1 L. The solution was placed for about 3 h under a temperature of about 55 °C to prepare a colloidal palladium activator labeled as A5.

### COMPARATIVE EMBODIMENT 1

The comparative embodiment 1 discloses a base colloidal palladium activator composition of the prior art.

The activator was substantial similar to that of EMBODIMENT 1, with the exception that 1.5 g vanillin was applied instead of glyoxylic acid.

The colloidal palladium activator was labeled as D1.

### COMPARATIVE EMBODIMENT 2

The comparative embodiment 2 refers to another palladium colloidal activator composition and a method for preparing the same.

3.422 mol sodium chloride were added into 750 ml deionized water to prepare a mixture. The mixture was stirred until dissolution. 0.24 mol concentrated hydrochloride, 0.020 mol isopropanol, and 0.5 mol urea were added to the mixture and stirred until dissolution to prepare a solution.

0.00028 mol palladium chloride was added in 70 ml deionized water having 0.36 mol concentrated hydrochloride to prepare a mixture. The mixture was stirred until dissolution. 0.00056 mol stannous chloride was added to the mixture and stirred for about 12 min to form a colloidal palladium mixture. The colloidal palladium mixture was added to the solution, and deionized water was added to make the volume of the solution to be 1 L. The solution was placed for about 3 h under a temperature of about 55 °C to prepare a colloidal palladium activator labeled as D2.

### EMBODIMENT 6

The embodiment discloses an activating method for a nonmetal surface.

A PI membrane with a size of 5 cm × 5 cm × 0.05 cm was immersed in a solution comprising about 1 mol/L sodium hydroxide, about 1 mol/L sodium carbonate and about 0.1 mol/L sodium dodecyl sulfonate, under a temperature of about 50 °C for about 8 min, and cleaned with clean water. Then the membrane was immersed in a PI adjusting agent (available from ZHUHAI SMART ELECTRONIC MATERIAL Co., LTD) having a temperature of about 35 °C, for about 7 min, then cleaned with clean water.

The PI membrane was dried by a fan dram, then immersed in A1 for about 3 min.

The PI membrane was cleaned with deionized water, and dispergated in a 10 vt% hydrochloride solution for about 5 min.

The PI membrane was cleaned with deionized water, and plated in 200 ml plating solution for about 20 min, where the plating solution comprises 0.040 mol/L copper sulfate, 0.107 mol/L EDTA, 0.0000237 mol/L potassium ferrocyanide, 0.00230 mol/L sodium dodecyl sulfonate, 0.000192 mol/L 2, 2'- bipyridine, and 0.0304 mol/L glyoxylic acid.

The PI membrane was cleaned with deionized water to form a plating element labeled as A6.

### EMBODIMENT 7-10

The embodiments 7-10 disclose activating methods for nonmetal surfaces.

The activating methods were substantial similar to that of EMBODIMENT 6, with the exception that A2-A5 were applied in stead of A1. The plating elements were labeled asA7-A10.

### COMPARATIVE EMBODIMENT 3-4

The activating method were substantial similar to that of EMBODIMENT 6, with the exception that D1-D2 were applied in stead of A1. The plating element was labeled as D3-D4.

### Testing

### 1. Activation life

50 ml A1-A5 and D1-D2 were separately placed in seven 50 ml colorimetric tubes, under room temperature (25 °C). The colorimetric tubes were not covered, and the time that colloidal palladium changed color was recorded. The results were shown in Table 1.

### 2. Activity

During the plating progresses of embodiment 6-10 and comparative embodiment 3-4, the following results were recorded: 1) initiating cycle, which was the time from the immersion of the PI membrane to foaming occurring on the surface of substrate; 2) sufficiently covering time, which is the time from the immersion of the PI membrane to the whole plating of the surface of the substrate. The results were shown in Table 1.
A6-A10 and D3-D4 were tested as below, and the results were shown in Table 2.

### 3. Thicknesses of the plating layers

Thicknesses of the plating layers were tested by a Membrane Testing Instrument (CMI900 available from Oxford instrument).

### 4. Adhesive strength

100 lattices with a size of 1 mm x 1 mm were cut on the plating layers. Transparent adhesive tape (type 600 available form Minnesota Mining &

Manufacturing Company) was bonded on the lattices and taken off as soon as possible, in a direction of an angle of about 60° with the surface of the layer. If no layers dropped, the adhesive strength was represented by 5B; if 0 to 5 % layers dropped, the adhesive strength was 4B; if 5 % to 15 % layers dropped, the adhesive strength was 3B; if 15 % to 35 % layers dropped, the adhesive strength was 2B; if 35 % to 65 % layers dropped, the adhesive strength was 1 B; if more than 65 % layers dropped, the adhesive strength was 0B.

### 5. Surface conditions of the layers

The surface conditions of the layers are observed by an SEM scan microscope (commercially available from SOHO-WORK Co, Ltd).

**Table 1**

| Samples | Life ( day ) | Initiation cycle ( s ) | Sufficiently covering time ( s ) |
|---|---|---|---|
| A1 | > 180 | 10 | 127 |
| A2 | > 180 | 9 | 113 |
| A3 | 157 | 15 | 138 |
| A4 | 140 | 15 | 135 |
| A5 | > 180 | 16 | 135 |
| D1 | 130 | 20 | 146 |
| D2 | 51 | 31 | 197 |

**Table 2**

| Samples | Thickness of the layers( µm ) | Adhesive strength | State of the surfaces |
|---|---|---|---|
| A6 | 1.1 | 4B | bright , no pinholes , no cracks |
| A7 | 1.2 | 5B | bright , no pinholes , no cracks |
| A8 | 1.0 | 4B | bright , no pinholes , no cracks |
| A9 | 0.7 | 4B | bright , no pinholes , no cracks |
| A10 | 0.9 | 4B | bright , no pinholes , no cracks |
| D3 | 0.6 | 3B | bright , no pinholes , no cracks |
| D4 | 0.4 | 2B | dark , pinholes , uneven thicknesses |

As shown in Table 1, colloidal palladium activator according to embodiments of the disclosure all had lives of more than 140 days. In addition, after surface treatments using colloidal palladium activator according to embodiments of the disclosure, the initiation cycles and sufficient covering time were less than those in the prior art.

Referring to Table 2, after surface treatments using colloidal palladium activator according to embodiments of the disclosure, the plating layers were uniform and flat, and had good adhesive strength with the nonmetal substrate.

## Claims

1. A colloidal palladium activator composition comprising:
colloidal palladium particles;
sodium chloride;
glyoxylic acid;
hydrochloride solution;
stannous chloride; and
a stabilizer.

2. The activator composition according to claim 1, wherein the colloidal palladium particles have a concentration of 0.0002 mol/L to 0.006 mol/L; the sodium chloride has a concentration of 2.567 mol/L to 3.765 mol/L; the glyoxylic acid has a concentration of 0.002 mol/L to 0.35 mol/L; the hydrochloride solution has a concentration of 0.12 mol/L to 0.96 mol/L; the stannous chloride has a concentration of 0.022 mol/L to 0.088 mol/L; the stabilizer has a concentration of 0.001 mol/L to 1 mol/L.

3. The activator composition according to claim 1 or 2, wherein the stabilizer is one or more selected from a group consisting of sodium stannate, carbamide, ascorbic acid, and the combinations thereof.

4. The activator composition according to any of the preceding claims, wherein the colloidal palladium particles have an average particle diameter of 80 nm to 300 nm.

5. The activator composition according to any of the preceding claims, wherein the activator further comprises a surface wetting agent.

6. The activator composition according to claim 5, wherein the surface wetting agent is one or more selected from a group consisting of isopropanol, methanol, ethanol, and the combinations thereof.

7. The activator composition according to claim 5 or 6, wherein the surface wetting agent has a concentration of 0.003 mol /L to 0.3 mol /L.

8. A method for preparing a colloidal palladium activator composition comprising steps of:
dispersing hydrochloride solution, stannous chloride, glyoxylic acid, and a stabilizer into sodium chloride solution to prepare an A solution;
dispersing palladium sodium into a hydrochloride solution and adding stannous chloride to prepare a B solution;
mixing the A and B solution to form the colloidal palladium activator composition.

9. An activating method for nonmetal surfaces comprising contacting a nonmetal substrate with a colloidal palladium activator composition according to any of claims 1 through 7.

10. The method according to claim 9, wherein the contacting process is performed under a temperature of 15 °C to 40 °C for 1 min to 5 min.

11. The method according to claim 9 or 10, wherein the nonmetal surface is pretreated by grease removal and rough treatments.

## Patentansprüche

1. Kolloidale Palladium-Aktivatorlösung, aufweisend:
kolloidale Palladiumteilchen;
Natriumchlorid;
Glyoxylsäure;
Hydrochloridlösung;
Zinn(II)-chlorid, und
einen Stabilisator.

2. Aktivatorlösung nach Anspruch 1, wobei die kolloidalen Palladiumteilchen eine Konzentration von 0,0002 mol/L bis 0,006 mol/L aufweisen; wobei das Natriumchlorid eine Konzentration von 2,567 mol/L bis 3,765 mol/L aufweist; wobei die Glyoxylsäure eine Konzentration von 0,002 mol/L bis 0,35 mol/L aufweist; wobei die Hydrochloridlösung eine Konzentration von 0,12 mol/L bis 0,96 mol/L aufweist; wobei das Zinn(II)-chlorid eine Konzentration von 0,022 mol/L bis 0,088 mol/L aufweist; wobei der Stabilisator eine Konzentration von 0,001 mol/L bis 1 mol/L aufweist.

3. Aktivatorlösung nach Anspruch 1 oder 2, wobei der Stabilisator einer oder mehrere ist, der/die aus einer Gruppe bestehend aus Natriumstannat, Harnstoff, Ascorbinsäure und deren Kombinationen ausgewählt ist/sind.

4. Aktivatorlösung nach einem der vorhergehenden Ansprüche, wobei die kolloidalen Palladiumteilchen einen durchschnittlichen Teilchendurchmesser von 80 nm bis 300 nm aufweisen.

5. Aktivatorlösung nach einem der vorhergehenden Ansprüche, wobei der Aktivator weiterhin ein Oberflächenbenetzungsmittel aufweist.

6. Aktivatorlösung nach Anspruch 5, wobei das Oberflächenbenetzungsmittel eines oder mehrere ist, das/die aus einer Gruppe bestehend aus Isopropanol, Methanol, Ethanol und deren Kombinationen ausgewählt ist/sind.

7. Aktivatorlösung nach Anspruch 5 oder 6, wobei das Oberflächenbenetzungsmittel eine Konzentration von 0,003 mol/L bis 0,3 mol/L aufweist.

8. Verfahren zur Herstellung einer kolloidalen Palladium-Aktivatorlösung, das die folgenden Schritte aufweist:
Dispergieren einer Hydrochloridlösung, von Zinn(II)-chlorid, Glyoxylsäure und eines Stabilisators in eine Natriumchloridlösung zur Herstellung einer A-Lösung;
Dispergieren von Palladium-Natrium in eine Hydrochloridlösung und Hinzufügen von Zinn(II)-chlorid zur Herstellung einer B-Lösung;
Mischen der A- und B-Lösung zur Ausbildung der kolloidalen Palladium-Aktivatorlösung.

9. Aktivierungsverfahren für Nichtmetalloberflächen, aufweisend das In-Kontakt-Bringen eines Nichtmetallsubstrats mit einer kolloidalen Palladium-Aktivatorlösung nach einem der Ansprüche 1 bis 7.

10. Verfahren nach Anspruch 9, wobei der Kontaktierungsprozess bei einer Temperatur von 15 °C bis 40 °C für 1 min bis 5 min durchgeführt wird.

11. Verfahren nach Anspruch 9 oder 10, wobei die Nichtmetalloberfläche durch das Entfernen von Schmiere und Raubehandlungen vorbehandelt wird.

## Revendications

1. Composition d'activation de palladium colloïdale, comprenant :
des particules colloïdales de palladium ;
du chlorure de sodium ;
de l'acide glyoxylique ;
une solution de chlorhydrate ;
du chlorure d'étain(II) ; et
un stabilisant.

2. Composition d'activation selon la revendication 1, les particules colloïdales de palladium ayant une concentration de 0,0002 mol/L à 0,006 mol/L ; le chlorure de sodium ayant une concentration de 2,567 mol/L à 3,765 mol/L ; l'acide glyoxylique ayant une concentration de 0,002 mol/L à 0,35 mol/L ; la solution de chlorhydrate ayant une concentration de 0,12 mol/L à 0,96 mol/L ; le chlorure d'étain(II) ayant une concentration de 0,022 mol/L à 0,088 mol/L ; le stabilisant ayant une concentration de 0,001 mol/L à 1 mol/L.

3. Composition d'activation selon la revendication 1 ou 2, dans laquelle le stabilisant est un ou plusieurs stabilisant/s sélectionné/s dans un groupe constitué de stannate de sodium, carbamide, acide ascorbique, et de leurs combinaisons.

4. Composition d'activation selon l'une des revendications précédentes, dans laquelle les particules colloïdales de palladium ont un diamètre de particule moyen de 80 nm à 300 nm.

5. Composition d'activation selon l'une des revendications précédentes, dans laquelle l'activateur comprend en outre un agent de mouillage de surface.

6. Composition d'activation selon la revendication 5, dans laquelle l'agent de mouillage de surface est un ou plusieurs agent/s sélectionné/s dans un groupe constitué d'isopropanol, méthanol, éthanol, et de leurs combinaisons.

7. Composition d'activation selon les revendications 5 ou 6, dans laquelle l'agent de mouillage de surface a une concentration de 0,003 mol/L à 0,3 mol/L.

8. Procédé de préparation d'une composition d'activation de palladium colloïdale, comprenant les étapes suivantes :
disperser la solution de chlorhydrate, le stannate de sodium, l'acide glyoxylique, et un stabilisant dans une solution de chlorure de sodium pour préparer une solution A ;
disperser le sodium de palladium dans une solution de chlorhydrate et ajouter du chlorure d'étain(II) pour préparer une solution B ;
mélanger la solution A et B pour former la composition d'activation de palladium colloïdale.

9. Procédé d'activation pour des surfaces non métalliques comprenant la mise en contact d'un substrat non métallique avec une composition d'activation de palladium colloïdale selon l'une des revendications 1 à 7.

10. Procédé selon la revendication 9, dans lequel le procédé de mise en contact est effectué à une température de 15 °C à 40 °C pendant 1 min à 5 min.

11. Procédé selon les revendications 9 ou 10, dans lequel la surface non métallique est prétraitée par l'enlèvement de graisse et par des traitements destinés à la rendre rugueuse.
